

## UNITED STATES PATENT OFFICE

2,129,748

## PROCESS OF TANNING WITH ALDEHYDES

Harold G. Turley, Moorestown, N. J., and Ian C. Somerville, Philadelphia, Pa., assignors to Rohm & Haas Company, Philadelphia, Pa.

No Drawing. Application June 20, 1936,  
Serial No. 86,338

7 Claims. (Cl. 149—5)

This invention relates to an improved process for tanning raw hides and skins, and particularly to simplification and improved control of the process of tanning with aldehydes.

5 It has long been known that raw hides and skins may be converted into leather by treatment with aldehydes, especially formaldehyde. In general the skins are prepared for formaldehyde tanning by first removing the hair with lime, 10 sodium sulfide, etc., after which the strong alkali is removed by the operation of bathing or puering. The resulting skins usually have a pH of the range of 7 to 9 and in this condition are ready for tanning with formaldehyde. In a second method the 15 skins, after unhairing, are pickled in a solution of sulfuric acid and salt, in which case it is necessary to neutralize the strong acid. This is accomplished either by the addition of a strong base, such as sodium hydroxide, or by employing the 20 well known action of buffer salts.

In establishing a uniform pH throughout the skins by these means frequently a long time is required to insure that the alkali penetrates the innermost fibers. The present invention is an 25 improvement in tanning skins prepared by the second of these methods whereby the neutralization is eliminated as an independent step and combined with the formaldehyde treatment.

It has been discovered that skins may be tanned 30 with aldehydes on the acid side of the iso-electric point and furthermore that the process of tanning may be carried out simultaneously with the step of adjusting the pH by adding to the aldehyde a sufficient quantity of buffer salt to establish the 35 proper pH, viz: 4.0 to 5.0.

It is an object of this invention to provide a 40 process for tanning pickled skins directly with aldehydes. It is a further object to provide a simple and easily controlled process thus insuring 45 uniformity and duplicability of results so that the usefulness of aldehyde tannage is greatly extended. Another object is to provide a simple aldehyde tannage which will permit the production of a good white leather and also of leather which has 50 an exceptionally smooth, fine grain.

The invention is carried out by treating the 55 pickled skins in a brine solution with a mixture of a buffer salt and an aldehyde capable of combining with the hide substance to produce leather.

50 In this way the pH is rapidly adjusted to the proper range and as a result the tanning reactions proceed more rapidly and uniformly than is possible by older methods. When the tanning is completed, the skins are thoroughly washed and fat- 55 liquored in the customary manner.

Various buffer salts may be used. These are principally the alkali metal salts of weak organic or inorganic acids such as acetic, citric, phosphoric, etc. The actual value of the pH used will vary somewhat with the type of skin, the desired 5 result and the time required for complete tannage and these factors must be considered in determining the amount and type of buffer necessary to produce the desired pH. The speed of aldehyde tanning increases as the numerical value of 10 the pH increases and for complete tannage with formaldehyde in about twenty-four hours the pH should be adjusted to 4.0 or slightly higher. Although we prefer to carry out this tanning process by the simultaneous treatment of the 15 pickled skin with the aldehyde and buffer salt, on the acid side of the iso-electric point, good results may also be obtained at pH values as high as 7.0. In the latter case the upper limit of the 20 pH will be determined by the appearance of the finished leather and should not be so high that a "drawn" or otherwise unsatisfactory grain is obtained. In all cases where the leather is to be subjected to further tanning by other agents, as for example according to the method of our 25 United States Patent No. 2,029,088, January 28, 1936, we prefer to carry out the simultaneous treatment of the skins with the aldehyde and buffer under such conditions that the tannage 30 takes place at a pH of 4.5 to 5.0.

Formaldehyde is the most suitable aldehyde for use in this process, particularly when white leather is desired. However, other reactive aldehydes such as crotonaldehyde may also be employed under the same conditions.

This invention is illustrated by the following examples but is not limited to the exact ingredients, proportions and temperatures shown as it may be otherwise practiced within the scope of 40 the appended claims.

*Example 1*

One hundred pounds of pickled kidskins was placed in a small drum with two hundred pounds of water and ten pounds of common salt. A solution of seven pounds of sodium citrate in fourteen pounds of 30% formaldehyde was run in. The pH of the liquid was 5.0. The skins were drummed for four hours and allowed to lie in the 45 liquor overnight. Next day they were thoroughly washed, set out and shaved, fatliquored with a mixture of five pounds of egg yolk and two and one-half pounds of neat's-foot oil, and horsed 50 overnight. Next day they were set out and hung to 55

dry in a cool room. When dry, they were sammied, staked out, and finished as usual.

*Example 2*

- 5 One hundred pounds of pickled calfskins was placed in a small drum with two hundred pounds of water and ten pounds of common salt. A mixture of eight pounds of disodiumphosphate and sixteen pounds of 30% formaldehyde was added.
- 10 The pH of the resulting liquor was 5.5. The skins were drummed for five hours and allowed to lie in the liquor overnight. Next day they were horsed, set out and shaved, thoroughly washed and fatliquored with four pounds of a good quality sulfonated neat's-foot oil. After horsing overnight, they were set out, crusted, and finished in the customary way.

*Example 3*

- 20 One thousand pounds of pickled steerhides, showing pH approximately three and one-half, was placed in a drum with two thousand pounds of water and one hundred pounds of common salt. While the drum was rotating, a solution of forty pounds of sodium acetate in one hundred twenty pounds of 30% formaldehyde was run in. The pH of the resulting liquor was 4.75. The skins were drummed for five hours and allowed to remain in the liquor overnight. Next day the drum was run one hour and the tanning supplemented by subsequent treatment with alum of forty per cent. basicity and a synthetic tanning agent.

*Example 4*

- 35 One hundred pounds of pickled capeskins was placed in a drum with two hundred pounds of water and ten pounds of common salt. Ten pounds of crotonaldehyde was added and the drum run five minutes, then a mixture of ten pounds of sodium acetate and one and one-half pounds of glacial acetic acid was added. The pH of the resulting liquor was 4.5. The drum was run intermittently for forty-eight hours, then the skins were washed thoroughly and fatliquored with twelve pounds of sulfonated cocoanut oil. After horsing overnight, they were hung to dry in a cool room, and finished as usual.

*Example 5*

- 50 One hundred pounds of pickled sheepskins was placed in a drum with two hundred pounds of water and ten pounds of common salt. A mixture of ten pounds of 37% formaldehyde, six pounds of disodium phosphate, and three-quarters of a pound of citric acid was added. The pH of the resulting liquor was 4.25. The drum was run intermittently for twenty-four hours. The liquor was drained off, the skins thoroughly washed, and fatliquored with two per cent. of sulfonated 60 olive oil. At the end of the fatliquoring operation, a white pigment was added. The skins were horsed overnight, set out, hung to dry in a cool place, and finished as usual.

The properties of leather prepared according 65 to these examples can be varied through wide limits by proper selection of pickled skins and by changing the conditions of processing. In all cases where formaldehyde is the tanning agent, white leather with a smooth grain is produced, 70 while crotonaldehyde gives a more creamy shade.

These reactions are carried out at ordinary temperatures for tannery operation, that is usually between 60° and 80° F. It is advantageous in some cases to raise the temperature towards the end of the tanning period, say as high as 120° F., when the rate of tanning is increased. Leather prepared according to these methods is resistant to water as hot as 180° F.

This process can be extended to a great variety of different types of pickled skins, as well as those specifically mentioned in the examples; for example, to furskins, buckskin, suede, calfskin, pigskin, reptile skins, horse hides and the like.

Since all special steps designed to prepare the pickled skins for aldehyde tannage, according to the usual practice, are eliminated by the present invention, a considerable amount of time is saved and a much simpler and more easily controlled method is provided.

We claim:

1. In the process of manufacturing leather the step which comprises treating the pickled skins directly, and without first depickling simultaneously with a buffer salt and an aldehyde capable of combining with the hide substance. 20

2. In the process of manufacturing leather the step which comprises treating the pickled skins directly, and without first depickling simultaneously with a buffer salt to adjust the pH to 4.0 to 5.0 and an aldehyde capable of combining with the hide substance. 25

3. In the process of manufacturing leather the step which comprises treating the pickled skins directly, and without first depickling simultaneously with an aldehyde capable of combining with the hide substance and a buffer salt in amounts sufficient to establish a pH approximately equal to that of the iso-electric point of the hide substance. 35

4. In the process of manufacturing leather the step which comprises treating the pickled skins directly, and without first depickling simultaneously with formaldehyde and a buffer salt in amounts sufficient to establish a pH approximately equal to that of the iso-electric point of the hide substance. 40

5. In the process of manufacturing leather the step which comprises treating the pickled skins directly, and without first depickling simultaneously with formaldehyde and a buffer salt in amounts sufficient to establish a pH of from 4.0 to 5.0. 50

6. In the process of manufacturing leather the step which comprises treating the pickled skins directly, and without first depickling simultaneously with formaldehyde and sodium acetate in amounts sufficient to establish a pH approximately equal to that of the iso-electric point of the hide substance. 55

7. In the process of manufacturing leather the step which comprises treating the pickled skins directly, and without first depickling simultaneously with formaldehyde and sodium citrate in amounts sufficient to establish a pH approximately equal to that of the iso-electric point of the hide substance. 65